

106-84

CROSS REFERENCE

EXAMINER

3

(No Model.)

P. H. GRIFFIN.

CORE FOR SASH WEIGHTS.

No. 254,126.

Patented Feb. 28, 1882.



Attest:

A. Barthel  
Chas. J. Hause

Inventor:  
P. Henry Griffin  
per Thos. S. Spagnus

Attest

106-84

254126

X R

# UNITED STATES PATENT OFFICE.

P. HENRY GRIFFIN, OF DETROIT, MICHIGAN.

## CORE FOR SASH-WEIGHTS.

SPECIFICATION forming part of Letters Patent No. 254,126, dated February 28, 1882.

Application filed September 7, 1881. (No model.)

*To all whom it may concern:*

Be it known that I, P. HENRY GRIFFIN, of Detroit, in the county of Wayne and State of Michigan, have invented an Improvement in Cores for Casting Sash-Weights, of which the following is a specification:

The nature of this invention relates to a new and useful core for casting sash-weights, by means of which a large saving of metal is obtained without deteriorating the value of the weight.

In the accompanying drawing a sash-weight provided with my improved permanent core is shown in vertical central section.

15 The molding is done in the usual manner, after which a core, A, is inserted into the mold and secured in place by any of the known and approved methods.

20 The core is made of sand, of the usual character for cores, mixed with silicate of soda, preferably in the proportion of twenty (20) parts of sand to one (1) part of silicate of soda, although I do not confine myself to the exact proportions named.

25 The mixture is pressed into a core-box to ob-

tain its proper shape, and is then dried in the usual manner before being placed in the mold. In casting, a thin shell, B, of iron is cast around the core, and the heat of the molten metal converts the core into a very hard substance resembling artificial stone of great density. The core varies but slightly in specific gravity from the iron surrounding it, and cannot be removed from the casting.

30 By the use of this core I am enabled to produce a weight wherein a large proportion of the metal is saved, the core becoming practically integral with the iron and differing therein from the ordinary cores, which become disintegrated by the heat of the molten metal and 40 are easily removed from the casting.

What I claim as my invention is—

A core for casting sash-weights, composed of sand and silicate of soda, as and for the purpose specified.

P. HENRY GRIFFIN.

Witnesses:

J. H. FLEMING,  
B. O'RORKE.